

## UNITED STATES PATENT OFFICE

2,614,078

## LUBRICATING COMPOSITIONS

Leonard R. Churchill, Cranford, N. J., assignor to  
 Tide Water Associated Oil Company, Bayonne,  
 N. J., a corporation of Delaware

No Drawing. Application December 10, 1949,  
 Serial No. 132,421

15 Claims. (Cl. 252—37.5)

1

The present invention relates to novel lubricating compositions and to the preparation thereof.

In the field of lubrication, extensive use has been made of compositions based upon a mineral oil, or fractions thereof, blended with sulfurized substances to impart certain desired properties to such oils that enhance the performance characteristics thereof in usage as lubricants for particular requirements. In example, the art is aware of the use of sulfurized substances blended with mineral oils for improving the oil with respect to extreme pressure properties, anti-welding, oiliness, etc. Thus, such sulfurized oil compositions have found extensive usage for many and varied lubricating operations and, particularly so as cutting oils, extreme pressure lubricants, etc. The art has resorted to various means for the preparation of such lubricants and, among such means, a widely used method is to incorporate sulfur into the compositions by blending a mineral oil with a sulfurized fatty oil. Although, by proper blending thereof, compositions may be prepared that possess properties enhancing usage of the lubricant where extreme pressure properties, improved cutting qualities, etc. are desired, such blends generally possess certain drawbacks that have retarded their more extensive usage for certain lubricating operations of specialized nature. For example, in some lubricating operations, it is highly desired that the lubricant be light in color and transparent and, in particular, such requirements are especially desired in cutting operations wherein visibility of the cutting tool and work is required during the cutting operation. For such usages, compositions comprising mineral oils blended with sulfurized materials have a drawback in that, although the mineral oil component may per se be light in color and transparent, blends thereof with sulfurized fatty oils are either too dark in color or are of non-transparent character, or both. The reason therefor is that fatty oils, upon sulfurization, usually provide dark colored and/or non-transparent products whereby, upon being blended with a mineral oil, the resulting blend possesses undesired characteristics as aforesaid for lubricating operations wherein lightness in color and transparency are desired characteristics for the lubricant. Hence, there is a need in the art for lubricating compositions based on a mineral oil blended with a sulfurized fatty oil that are light in color, transparent and stable against darkening during storage and usage while possessing the desired properties imparted to the mineral oil by blending thereof with

2

the sulfurized fatty oil. A major object of the present invention is to provide lubricating compositions that are devoid of the aforesaid undesirable characteristics generally possessed by sulfurized fatty oil-containing-mineral oil compositions.

Generally speaking, the present invention is based upon the discovery that a mineral oil blended with a sulfurized fatty oil, and which blend is dark colored and/or is objectionably non-transparent due to the presence of the sulfurized fatty oil therein, may be converted to suitable light colored, transparent lubricating compositions by subjecting such blends to an oxidation treatment as described more fully hereinafter.

As is apparent from the foregoing, the lubricating compositions embodied herein contain, as essential ingredients, a mineral oil possessing characteristics suitable for the contemplated usage of the composition, and a sulfurized fatty oil that, upon being blended with the mineral oil, substantially darkens the mineral oil and/or provides a blend of non-transparent character. Hence, and although it is not intended that the present invention be limited as to the method for preparation of the sulfurized fatty oil-mineral oil blends to be subjected to treatment in accordance with this invention, an efficacious method is to simply dissolve the sulfurized fatty oil, in desired concentration, in the mineral oil by use of means such as heating, agitation, or otherwise, as desired.

With reference to the mineral oil component of the compositions embodied herein, a wide range of mineral oils may be employed, the particular physical characteristics thereof being dependent upon the particular lubricating operation for which the composition is to be employed. Hence, the invention contemplates use of mineral oils that possess lubricating properties and which may be derived from any of a variety of petroleum crudes including paraffinic, naphthenic and mixed crudes. Although it is not intended that the present invention be limited to lubricants for usage in cutting operations, the compositions contemplated herein find particular utility therefor, and hence, for purposes of illustration, the invention is described with particular reference thereto. For such cutting oil usage, the compositions contemplated herein desirably contain a mineral oil that possesses lubricating properties, a viscosity within the range of about 50 to 900 SUS at 100° F., and a flash point of at least 300° F. More preferably, and particularly for contemplated usage in light cutting operations, the

mineral oil component employed desirably possesses a viscosity of about 50 to 300 SUS at 100° F., has a flash point of over 300° F., and is light in color, e. g., having an ASTM color value of about 1 to 3 or lighter.

With reference to the second essential component of the compositions embodied herein, i. e., a sulfurized material, the invention contemplates use of fatty oils that, upon sulfurization, are dark-colored and/or are of non-transparent character and which, upon blending with a mineral oil, dark and/or impart non-transparent characteristics to the mineral oil. Although the invention contemplates broadly the use of fatty oils that possess such characteristics upon sulfurization, suitable illustrations of such fatty oils include sperm oil, lard oil, and the like. Depending upon the particular type of fatty oil employed, the amount of sulfur combined therewith may be varied but, for most purposes, sulfurized fatty oils containing about 5 to 15% sulfur are employed. The art is aware of various methods for preparation of sulfurized fatty oils and, hence, a detailed description thereof is not deemed necessary herein. However, for purposes of illustration without intent of limitation, and using sperm and lard oils to illustrate specific embodiments, sulfurization thereof to provide substances suitable for practicing this invention may be effected by preparing a mixture of the fatty oils with, for example, about 10% by weight thereof of sulfur flour, and heating the mixture with agitation at about 320 to 400° F. for about 1½ to 2 hours.

Depending upon the intended usage of the compositions embodied herein, the amount of sulfurized fatty oil blended with the mineral oil may be varied over a wide range. Generally speaking, however, the compositions contemplated herein comprise a suitable mineral oil blended with sulfurized material in an amount normally imparting perceptible darkening of color which usually amounts to from about 1% to about 100%, based on the weight of the mineral oil, of the sulfurized fatty oil. Thus, for certain heavy duty lubricating operations and wherein a high concentration of sulfur may be desired in the blended composition, the sulfurized fatty oil may be used in a ratio as high as equal parts by weight with the mineral, whereas, for lighter duty lubricating operations, the amount of sulfurized fatty oil employed is usually from about 1% to about 10%, or about 1% to about 5%, by weight of the mineral oil. More specific illustrations include a suitable mineral oil blended with about 2 to 5% of sulfurized fatty oil, e. g., sperm oil or lard oil containing about 10% of sulfur in non-corrosive form.

In preparing the compositions embodied herein, a blend of the mineral oil and sulfurized fatty oil, and which blend is of undesirable dark color and/or of non-transparent character due to the presence of the sulfurized fatty oil, is subjected to a controlled oxidation treatment to substantially reduce the color of the blend and to effect conversion thereof to a transparent composition that has enhanced utility for lubricating operations wherein lightness in color and transparency of the lubricant are desired. In accordance with this invention, such dark-colored and/or non-transparent blends are treated with a free oxygen-containing gas, in the presence of an oxidation catalyst, until the dark-colored and/or non-transparent blend is substantially reduced in color and converted to a transparent composition. Preferably, the treatment is continued

until the color characteristics of the dark-colored sulfurized fatty oil-mineral blend are similar to that of the mineral oil per se. Thus, the treatment may be employed to substantially, or fully, remove the color characteristics imparted to the mineral oil by the sulfurized fatty oil while maintaining the desired characteristics imparted to the mineral oil by the sulfurized fatty oil and the performance thereof for lubricating operations.

In practicing this invention, the oxidation treatment is preferably effected by blowing or otherwise intimately contacting the sulfurized fatty oil-mineral oil blend with a free-oxygen containing gas, examples of which include air, oxygen, mixtures thereof, etc. in the presence of a suitable oxidation catalyst until the desired conversion of the dark-colored blend is obtained. Although the catalysts employed may be of many and varied types of substances having catalytic properties for oxidation purposes, especially preferred substances are metal soaps of organic acids, e. g., of fatty acids such as oleic, stearic, and the like, and naphthenic acids. In more specific embodiment, suitable catalysts include oil-soluble soaps of polyvalent metals, e. g., such as lead, cobalt, manganese, etc., and more preferably the naphthenic acid soaps thereof which possess activity as oxidation catalysts. The catalysts may be used in small amounts sufficient to catalyze the oxidation and, or if desired, in amounts in excess thereof. For example, larger amounts may be desired when the catalyst, in addition to catalyzing the oxidation treatment, also imparts some desired characteristic or characteristics to the blend. As the art is aware, metal soaps are oftentimes desired ingredients in lubricating compositions as they generally impart improved load-carrying properties thereto. Examples of such soaps include suitable fatty acid and naphthenic acid soaps of metals and, especially of metals such as lead, cobalt, manganese, etc. Thus, when it is desired to provide lubricating compositions embodied herein which also contain a metal soap, the metal soaps preferably employed are those that also possess activity as oxidation catalysts. Thus, and in accordance with specific embodiments of this invention, blends may be prepared that contain the soap in desired proportion, e. g., about 0.5 to 10% based on the weight of the composition, sufficient to impart desired properties to the blend and, in which case the soap functions as the catalyst in the oxidation treatment and also provides lubricating compositions possessing desired properties imparted thereto by such soaps and sulfurized fatty oils.

In order to further describe the invention, several examples are set forth hereinafter showing illustrative, but not limitative, embodiments of the invention.

#### Example I.

Several blends were prepared by dissolving 1% by weight of lead naphthenate in a light-colored transparent non-viscous neutral oil having an ASTM color value of about 2, a viscosity of from 50 to 60 SUS at 100° F., a flash point of over 300° F., and derived from a paraffinic base petroleum crude. The resulting blends had an ASTM color value of about 2½, thus evidencing that the lead naphthenate had not substantially increased the color value of the oils. Three percent by weight of a non-corrosive sulfurized sperm oil (10% sulfur) was dissolved in the lead naphthenate-

mineral oil blends whereupon dark-reddish-black colored blends were obtained having ASTM color values of about 5 to 5½. Each of the dark-colored blends was heated to 160° to 180° F. and treated by bubbling air therethrough. Upon such treatment for periods of about 8 to 24 hours, during which no evidence of precipitation was observed, the dark-colored blends were reduced in color value to about 2½, or even lighter in some instances, i. e., the sulfurized fatty oil blends were reduced in color to ASTM values at least as low as that of the compositions minus the color-imparting sulfurized fatty oil.

In order to illustrate the importance of using an oxidation catalyst, a dark-colored composition was prepared consisting of 97% of a mineral oil as described in this example blended with 3% of the sulfurized sperm oil, and, hence, devoid of the oxidation catalyst. The composition was blown with air under the same conditions as the aforesaid lead naphthenate-sulfurized fatty oil-containing composition without any significant decolorization being effected upon treatment for 192 hours.

*Example II*

A composition was prepared by blending a mineral oil, as described in Example I, with 1% of manganese naphthenate, and 3% of sulfurized sperm as described in Example I. Upon treatment of the resulting dark-colored blend, in a manner similar to that described in Example I, the blend was reduced in color to substantially the same color value as the mineral oil itself.

*Example III*

A composition was prepared by blending a mineral oil, as described in Example I, with 1% of lead naphthenate and 3% of non-corrosive sulfurized lard oil (10% sulfur). The resulting blend, reddish-black in color, was treated with air in the manner described in Example I, and similar thereto, the dark-colored blend was reduced in color to substantially the same color value of the mineral oil itself.

The light-colored transparent compositions embodied herein, resulting from treatment of dark-colored sulfurized fatty oil-mineral oil blends as aforescribed, are highly stable against reversion to dark-colored compositions as observance of the treated compositions over extended periods of time, e. g., two weeks or more, has revealed that no significant, if any, color changes occurred. Moreover, and in addition to effecting the desired conversion to light-colored, transparent compositions, treatment of the sulfurized fatty oil-mineral oil blends in accordance with this invention generally improves the wetting properties of the blends and, as those in the art are aware, such an improvement is highly desired in lubricating compositions, especially in the use thereof for metal cutting and extreme pressure lubricating operations.

Although the foregoing examples illustratively set forth the improvements obtained by practicing this invention with reference to compositions of certain specific ingredient concentrations, it should be understood that the invention is not to be considered as limited thereto with respect to ingredient concentrations, treatment conditions, etc. As to ingredient concentrations, these may be varied over rather wide ranges as described hereinbefore. With reference to the treatment, and especially the time period necessary for reducing the color of the sulfurized fatty

oil-containing blends to desired color values, the time required is dependent upon consideration of several factors including particular concentrations of ingredients employed, the desired reduction in color value, the amount of free-oxygen-containing gas maintained in contact with the blend under treatment, the extent to which agitation of the blend is maintained during the treatment to effect intimate contact of the blend with the free-oxygen-containing gas, and the like. It is apparent, therefor, that the present invention in generic aspect relates to controlled oxidation of the dark-colored sulfurized fatty oil-containing mineral oil compositions in the presence of a suitable oxidation catalyst for a period of time sufficient to effect conversion of the dark-colored blends to light-colored, transparent compositions.

As far as I am aware, the compositions embodied herein are not only novel but are the result of the use of a treatment for dark-colored sulfurized fatty oil-mineral oil blends that, in an unexpected manner, effects conversion of such dark-colored and/or non-transparent blends to light-colored, transparent compositions. Although the reasons underlying the results obtained by practice of this invention are not fully understood, it appears that by use of mineral oil blends of the sulfurized fatty oils, the controlled treatment disclosed functions to selectively oxidize and substantially reduce the color characteristics of color-imparting components of the sulfurized fatty oils. An important observation made during the investigation upon which the present invention is based is that by treatment of the blends contemplated herein with a free-oxygen-containing gas in the presence of an oxidation catalyst, and even though the amount of catalyst used may be in excess (e. g., as in Examples I to III) of that required to perform the catalytic function, the desired results have been provided without formation of precipitates during the treatment, thus indicating that selective oxidation of color-imparting bodies of the sulfurized fatty oils apparently occurs rather than undesired reactions between ingredients in the compositions to the extent of formation of insoluble reaction products that would tend to precipitate during the oxidation treatment.

Obviously, many modifications and variations of the invention, as hereinbefore set forth, may be made without departing from the spirit and scope thereof and, therefore, only such limitations should be imposed as are indicated in the appended claims.

I claim:

1. In the preparation of lubricating compositions by blending a mineral oil with a sulfurized fatty oil that substantially increases the color characteristics of said mineral oil, the improvement which comprises subjecting said blend to controlled contact with a free-oxygen containing gas in the presence of a metal salt of an organic acid possessing activity as an oxidation catalyst for a period of time sufficient to substantially decrease the color characteristics imparted to said blend by said sulfurized fatty oil.

2. A method, as defined in claim 1, wherein the free oxygen-containing gas is a member from the group consisting of air and oxygen.

3. In the preparation of lubricating compositions by blending a mineral oil with a sulfurized fatty oil that substantially increases the color characteristics of said mineral oil, the improve-

ment which comprises subjecting said blend in controlled contact with a gas from the group consisting of air and oxygen in the presence of a metal soap from the group consisting of polyvalent metal soaps of fatty acids and naphthenic acids possessing activity as oxidation catalysts for a period of time sufficient to substantially decrease the color characteristics imparted to said blend by said sulfurized fatty oil.

4. A method, as defined in claim 3, wherein the sulfurized fatty oil is sulfurized sperm oil.

5. A method, as defined in claim 3, wherein the sulfurized fatty oil is sulfurized lard oil.

6. Method for reducing the color characteristics of mineral oil compositions having dissolved therein a sulfurized fatty oil that substantially increases the color characteristics of said mineral oil which comprises subjecting said sulfurized fatty oil-containing mineral oil composition to controlled contact with a free-oxygen containing gas in the presence of a metal salt of an organic acid possessing activity as an oxidation catalyst for a period of time sufficient to substantially reduce the color characteristics imparted to said composition by said sulfurized fatty oil.

7. As a new composition, a mineral oil blended with a sulfurized fatty oil that substantially increases the color characteristics of said mineral oil, and which blend has been subjected to controlled contact with a free oxygen-containing gas in the presence of a metal salt of an organic acid possessing activity as an oxidation catalyst for a period of time sufficient to substantially reduce the color characteristics imparted to said mineral oil by said sulfurized fatty oil.

8. A composition, as defined in claim 7, wherein the free oxygen-containing gas is a member from the group consisting of air and oxygen.

9. A composition, as defined in claim 7, wherein the sulfurized fatty oil is sulfurized lard oil.

10. A composition, as defined in claim 7, wherein the oxidation catalyst is a polyvalent metal soap of an acid from the group consisting of fatty acids and naphthenic acids.

11. A composition, as defined in claim 7, wherein the sulfurized fatty oil is sulfurized sperm oil.

12. A composition, as defined in claim 7, which comprises a mineral oil in major amount based on the weight of said composition.

13. A composition, as defined in claim 12, wherein the sulfurized fatty oil is sulfurized sperm oil and the catalyst is a naphthenic acid salt of a metal from the group consisting of lead, manganese, and cobalt.

14. As a new composition, a mineral oil blended with a sulfurized fatty oil that substantially increases the color characteristics of said mineral oil, and which blend has been subjected to controlled contact with a free oxygen-containing gas in the presence of a naphthenic acid soap of a metal from the group consisting of lead, manganese, and cobalt for a period of time sufficient to substantially reduce the color characteristics imparted to said mineral oil by said sulfurized fatty oil.

15. A composition comprising a mineral oil in major amount based upon the weight of said composition, a sulfurized fatty oil in an amount sufficient to substantially increase the color characteristics of said mineral oil, and a small amount of an oil-soluble metal salt of naphthenic acid that possesses activity as an oxidation catalyst, said composition being characterized by having been subjected to controlled contact with a free-oxygen containing gas for a period of time sufficient to substantially decrease the color characteristics imparted thereto by said sulfurized fatty oil.

LEONARD R. CHURCHILL.

#### REFERENCES CITED

The following references are of record in the file of this patent:

#### UNITED STATES PATENTS

| 40 | Number    | Name          | Date          |
|----|-----------|---------------|---------------|
|    | 2,023,768 | Otto          | Dec. 10, 1935 |
|    | 2,070,567 | Adams         | Feb. 16, 1937 |
|    | 2,179,060 | Smith         | Nov. 7, 1939  |
|    | 2,240,054 | Richardson    | Apr. 29, 1941 |
|    | 2,301,794 | Proell et al. | Nov. 10, 1942 |